

3,234,160

## PROCESS FOR MAKING POLYVINYL ALCOHOL FIBERS HAVING IMPROVED PROPERTIES

Kanji Matsubayashi, Kurashiki, Japan, assignor of one-fourth to Air Reduction Company, Incorporated, New York, N.Y., a corporation of New York, and three-fourths to Kurashiki Rayon Co., Ltd., Okayama Prefecture, Japan, a corporation of Japan

No Drawing. Filed July 15, 1960, Ser. No. 42,997  
Claims priority, application Japan, July 16, 1959,

34/22,797

3 Claims. (Cl. 260—29.6)

This invention relates to a method for producing fibers of polyvinyl alcohol which have improved dyeability.

As is well known, fibers derived from polyvinyl alcohol, known commercially as Vynylon, and produced by spinning from an aqueous solution of polyvinyl alcohol followed by formalization after heat-treatment, have insufficient dyeability, and many attempts have been made to improve this property. Although the problem of providing sufficient dyeability in the case of acid wool dyes and direct cotton dyes has been generally solved by methods such as animalization, these methods are accompanied by disadvantages such as the fact that the introduced basic nitrogen tends to cause yellowing upon heating or prolonged use of the fiber. Even these methods, therefore, leave substantial room for improvement. Basic dyes heretofore in use are bright in color, but they lack light fastness, and similar desirable characteristics and they are not, therefore, of commercial importance at this time. Cation dyes have, however, recently been proposed as dyes for acrylic fibers such as Orlon, and the like, and these dyes have been found to have an improved light fastness. These dyes have thus become of substantial commercial importance. It is believed that these dyes have an affinity for the acid group contained in the fiber. In connection with fibers of polyvinyl alcohol, for example, as shown in the co-pending application of Keniche Tanabe et al., Ser. No. 787,386, filed January 19, 1959, now Patent No. 3,023,182, it has been found that their affinity for basic dyes can be increased by spinning the fibers from a mixture of polyvinyl alcohol and a water-soluble polymer containing a sulfo group. However, it has become apparent that when such a water-soluble polymer is used, if acetalization is carried out by means of aromatic aldehydes, such as benzaldehyde, naphthaldehyde, and the like, which bring about a marked increase in the elastic recovery of the fibers, the dyeability drops substantially. A decrease in dyeability is also noted when the fibers are subjected to hot stretching, which is effective to increase the strength and elasticity of the fibers.

It is thus an object of this invention to provide a process for producing fibers of polyvinyl alcohol having high hot-water resistance and heat-resistance and desirable mechanical properties at least equal to known commercial polyvinyl alcohol fibers, yet characterized by a particularly high dyeability, particularly with respect to silk dyes, such as basic dyes, cation dyes, and the like, and with respect to dyes proposed for acrylic-type fibers.

In accordance with this invention, spinning of fibers is effected from a spinning fluid prepared by dispersing in a water solution of polyvinyl alcohol an emulsion or fine powder of a water-insoluble polymer containing an acid radical such as a carboxyl group of a sulfo group.

I have discovered that when a spinning fluid is prepared by dispersing in a polyvinyl alcohol solution an emulsion or fine powder of water-insoluble polymers containing acid groups, even when the fiber is subsequently made hydrophobic by treatments such as benzalization, and the like, no decrease in dyeability takes place and the fibers exhibit excellent dyeability for the above-mentioned

dyes. Furthermore, the larger the particle size of the solid particles of polymer and the greater the degree of hot stretching, the better the dyeability.

The reason for the foregoing results are not fully understood. However, it is presumed that, in the case of such solid particles, the larger the size of the particles, the less the particles are affected by the polyvinyl alcohol molecule or its benzalized portion, with the result that the dyestuff can more easily permeate the fibers. In any case, since there is an existing need for polyvinyl alcohol or vynylon fibers having excellent elastic recovery and dyeability, this invention is of substantial significance since it makes it possible to achieve this objective and to provide the desired fibers conveniently and economically.

The emulsion or fine powder of the polymers containing acid groups suitably used in accordance with the present invention is conveniently manufactured by various methods. For example, polymerizable monomers containing acid groups such as a carboxyl groups or a sulfo group, or their salts such as their sodium salts, ammonium salts, and the like, e.g. acrylic acid, methacrylic acid, crotonic acid, vinyl sulfonic acid, allylsulfonic acid, styrenesulfonic acid, and their salts, are polymerized by emulsion polymerization or suspension polymerization techniques. The desired water-insoluble polymer, can also be obtained by suspension or emulsion copolymerization of the above-characterized monomers with other polymerizable monomers such as vinyl chloride, allyl chloride, vinylidene chloride, vinyl benzoate, allyl acetate, styrene, butadiene, divinylbenzene, methyl acrylate, methyl methacrylate, acrylonitrile, methyl vinylketone, and the like. Emulsion polymerization, or suspension polymerization are easily effected by conventional means, using anionic surface active agents or non-ionic surface active agents as emulsifier, and using various water-soluble polymers such as polyvinyl alcohol, gelatin, and the like, as protective colloids, if desired. The particle size of the emulsified or suspended polymer is suitably from 0.01 $\mu$  to a few  $\mu$ , e.g. 10 $\mu$ . The desired emulsion or fine powder can also be produced by dissolving a water-insoluble polymer having an acid group, e.g. polymers formed from the above-mentioned monomers, in an organic solvent, and the solution is then dispersed in water in the presence of a surface active agent or protective colloid, and then the organic solvent is removed by distillation.

Use can also be made of polymers having acid groups, which are obtained by introducing the acid group by chemical reaction effected upon a polymer having a reactive group which can be converted to an acid group. For example, by partial saponification of methyl polyacrylate, a water-insoluble polymer having an acid group can be obtained. This reaction can be carried out after the formation of an emulsion of the polymer or chemical reaction may be carried out prior to the formation of the emulsion, the emulsion of the converted polymer then being prepared by the above-mentioned method.

Water-insoluble polymers containing an acid group are also suitably formed in emulsified or in finely divided powder form by acetalizing a water-soluble polymer, such as polyvinyl alcohol, by means of aldehydes containing acid groups such as glyoxylic acid, carboxy-acetaldehyde, azelaic aldehyde, sulfo-acetaldehyde, disulfo-acetaldehyde,  $\alpha$ -, or  $\beta$ -propion-aldehyde,  $\alpha$ -,  $m$ -, or  $p$ -sulfobenzaldehyde, sulfonaphthaldehyde, and the like. Simultaneously with such acetalization, or before or after it, acetalization of the polymer may be effected by means of aldehydes having no acid radical such as formaldehyde, butyraldehyde, benzaldehyde, and the like, to produce water-insoluble polymers for use in accordance with this invention. In forming emulsions of polymers by this last-named procedure, it is advantageous to effect the reac-

tion with high-speed agitation or to add various surface-active agents or water-soluble polymers, and the like to the reaction mixture to serve as emulsifiers or protective colloids. In accordance with this method, particle sizes ranging from  $0.1\mu$  to  $10\mu$ , can easily be obtained. In the case of these acetalized polyvinyl alcohols, the previously mentioned methods for dispersing polymers in water may also be used to form the emulsion.

Acetalization by means of aldehydes containing no acid groups, such as those mentioned above, may also be effected upon polyvinyl alcohol derivatives containing these acid groups or upon copolymers composed principally of vinyl alcohol, e.g. saponified copolymers of crotonic acid and vinyl acetate, and the like, in order to insolubilize the polymers or copolymers. Similarly, acetalization may be effected by means of aldehydes having no acid groups upon polyvinyl alcohol derivatives which have functional groups which are easily convertible into acid groups by chemical reaction, or upon copolymers principally composed of vinyl alcohol and containing such convertible groups, such as the copolymerization-saponification product of allyl chloride and vinyl acetate, in order to insolubilize such polymers. The reaction to effect introduction of acid groups, e.g. sulfonation, effected by the action of sodium sulfite on halogens, such as chlorine, is suitably carried out while the polymer is in emulsified or finely-divided form.

It is preferable to use aldehydes containing acid groups for the introduction of the acid group into polyvinyl alcohol, but such groups may be introduced by other reactions applied to polyvinyl alcohol, e.g. oxidation by means of an oxidizing agent such as potassium permanganate, and the like, sulfo ethyl-etherification by means of vinylsulfonic acid, hydrolysis after carbamoyl-ethyl-etherification by means of acrylamide, and like known other methods for the introduction of an acid group.

In addition, the product of reaction to introduce an acid group into water-insoluble particles such as starch, e.g. etherification with monochloroacetic acid, can also be used. In either case, as the result of the introduction of an acid group such as the carboxyl or the sulfo group, a suitable hydrophilic quality and electrical repulsion are imparted to the polymer particles, so that the emulsion or finely-divided powder of the polymers used has enhanced stability in water and in admixture with polyvinyl alcohol, and when they are dispersed in the spinning fluid, their stability is further increased so that the spinning fluid is easily and readily filtered to facilitate spinning. However, when the content of the acid group is too high, it may become difficult to insolubilize the polymers by reason of pronounced hydrophilic quality provided by the high acid group content. It is difficult to define the optimum range of the acid group content because it depends upon the hydrophobic qualities of the particular polymer and the hydrophilic quality of the particular acid group, but the range of 1-70 mol percent has been found to be suitable, mol percent being based on the polymer containing the acid group. A suitable ratio for mixing these polymers with polyvinyl alcohol to form a spinning fluid is 0.1-10 mol percent. When this ratio is used, a marked increase is noted in the dyeability of the resulting fibers with respect to cation dyes and basic dyes. Moreover, any decrease in hot-water resistance, heat-resistance, mechanical properties, and the like is held to a minimum. The particle size of the polymer is suitably within the range of  $0.01\mu$ - $10\mu$ .

In accordance with the present invention, it is possible, without difficulty, to obtain solid particles having such particle diameters of  $1\mu$ - $30\mu$ .

When the particle diameter is too large, the percentage of broken fibers and nappy fibers increases, resulting in a yarn of poorer mechanical properties. Thus, it is desirable for the particle diameter to be below  $30\mu$ .

It is possible to carry out spinning by means of the spinning fluid prepared by dispersing an emulsion or a fine powder of the polyvinyl alcohol derivatives with polyvinyl alcohol by the method of this invention, with the addition of various types of water-soluble polymers such as soluble starch, polyvinylpyrrolidone, aminoacetalized polyvinyl alcohol, various kinds of pigments such as titanium oxide, and acids, alkalies, and salts such as sodium sulfate, and the like. Accordingly, it is possible to simultaneously effect improvements in the transparency and in the form of the cross-section of the fibers, particularly when the fibers are formed by wet spinning.

The fibers spun by the method of this invention may be subjected to thermal elongation, i.e. hot-stretching, heat-treatment and insolubilization treatments in the same manner as fibers formed solely from ordinary polyvinyl alcohol. For effecting insolubilization, acetalization by means of aliphatic, aromatic or aralkyl aldehydes is suitably employed. Suitable aldehydes for this purpose include formaldehyde, acetaldehyde, chloroacetaldehyde, butyraldehyde, nonylaldehyde, benzaldehyde, monochlorobenzaldehyde, 1-naphthaldehyde, glyoxal, malonaldehyde, glutaraldehyde, terephthalaldehyde, and like aliphatic, aromatic and aralkyl aldehydes. The fibers may also be subjected to treatments with inorganic reagents such as titanification, and chroming. Various other known insolubilization treatments may also be employed.

The invention will be further understood from the following specific examples of practical application. However, it will be understood that these examples are not to be construed as limiting the scope of the present invention in any manner. In these examples, all parts are by weight, unless otherwise indicated.

#### Example 1

A mixture of methyl acrylate (77.4 g.), acrylic acid (7.2 g.), caustic soda (2 g.), polyvinyl alcohol (17 g.), the anion dispersant,  $\alpha$ -sodium sulfosuccinic diethyl ester (4 g.), potassium persulfate (0.5 g.), sodium bisulfite (0.3 g.) and water (500 g.) was stirred at  $60^\circ$  C. for 4 hours to effect emulsion polymerization. Unreacted substances were removed by steam distillation and dialysis, and an emulsion of 9.1% concentration was obtained in a yield of 81%. This emulsion was mixed with 20% of polyvinyl alcohol, and a spinning fluid having a total polymer concentration of 15% was prepared. The fluid was wet-spun into a coagulation bath of sodium sulfate in conventional manner. The fibers thus produced were stretched by 100% at  $230^\circ$  C., and shrunk by 20% at  $235^\circ$  C. The fibers were then formalized in a bath consisting of formaldehyde (5%), sulfuric acid (15%), and sodium sulfate (15%) at  $70^\circ$  C. for one hour. The degree of formalization was 38 mol percent. These fibers underwent shrinkage of 3.8% when treated in boiling water for 30 min. The temperature at which a 10% shrinkage occurred in air (softening point) was  $210^\circ$  C. The fiber strength was 4.8 g./denier. When dyed with the basic dye methylene blue (4%) and acetic acid (1%) (percentages based on the weight of fiber) at  $80^\circ$  C. for 2 hours, the dye was almost completely absorbed and a saturated blue color was obtained.

#### Example 2

A mixture composed of 688 g. vinyl acetate, 172 g. crotonic acid (20 mol percent of both monomers), partially saponified polyvinyl acetate of a degree of saponification of 85 mol per (150 g.), polyoxyethylene (20 mol percent), lauryl ether (86 g.), hydrogen peroxide (4 g.), sodium tartarate (1 g.) and water (4 l.), was subjected to emulsion polymerization at  $60^\circ$  C. for 3 hours, and was purified by steam distillation. The emulsion thus obtained was mixed with 25% of polyvinyl alcohol, and wet-spinning was effected in the manner described in Example 1. The result was as satisfactory as that realized by spinning a water solution of polyvinyl alcohol alone, and the

spinning operation could be performed satisfactorily. The fibers produced were heat-treated as described in Example 1. After heat-treatment as described in Example 1, some of the fibers were formalized by the procedure of Example 1 (Sample I). The remaining fibers were benzalized in a water solution containing benzaldehyde (2%), sulfuric acid (10%), and methanol (30%) at 60° C. for one hour (Sample II). For the purpose of comparison, fibers were spun from a conventional polyvinyl alcohol spinning bath to which polyacrylic acid (5% based on polyvinyl alcohol), and caustic soda (50 mol percent base on polyacrylic acid) were added, and after heat-treatment as described above, the fibers were formalized (Sample III) or benzalized (Sample IV), formalization and benzalization being effected by the procedures used in producing Samples I and II, respectively.

For the purpose of further comparison, additional fibers were spun from a water solution of polyvinyl alcohol alone and these fibers were heat-treated and formalized (Sample V) or benzalized (Sample VI) as described above. The various properties of these several fibers are set forth below:

| Properties                                                            | Samples          |                  |                  |                |                |                |
|-----------------------------------------------------------------------|------------------|------------------|------------------|----------------|----------------|----------------|
|                                                                       | I                | II               | III              | IV             | V              | VI             |
| Carboxyl content (Based on the entire polymer content) (mol percent). | 2.26             | 2.26             | 2.98             | 2.98           |                |                |
| Acetalization.                                                        | Formalization.   | Benzalization.   | Formalization.   | Benzalization. | Formalization. | Benzalization. |
| Degree of Acetalization (mol percent)                                 | 39               | 22               | 41               | 23             | 37             | 21             |
| Shrinkage in boiling water (percent)                                  | 3.5              | 7.5              | 6.0              | 9.1            | 3.0            | 6.5            |
| Strength (g./denier)                                                  | 4.6              | 4.4              | 4.1              | 4.0            | 4.9            | 4.6            |
| Elasticity, (percent) (at 3% Elongation)                              | 55               | 75               | 54               | 74             | 56             | 78             |
| Dyeability <sup>1</sup>                                               | Saturated color. | Saturated color. | Saturated color. | Light color.   | Light color.   | Stained.       |

<sup>1</sup> Dyed with 4% Sevron Green B, or 4% Sevron Red B and 1% acetic acid (percentages based on the weight of fiber), at 80° C. for 2 hours.

Sample V, and particularly Sample VI, which is ordinary Vynylon, did not exhibit a dyeability of any practical value with the above-mentioned Sevron Colors, whereas in the case of the formalized Sample III, a saturated color was obtained, but in the benzalized Sample IV, which exhibited excellent elasticity, only a light color was obtained. In Samples I and II, produced by the method of this invention, a saturated color of practical value was obtained, and particularly in the case of benzalized Sample II, the elasticity was also fully satisfactory.

#### Example 3

An aqueous solution containing polyvinyl alcohol (3%), formaldehyde (1%) and sulfuric acid (50%) was reacted at 50° C. for 2 hours with agitation at 1,000 r.p.m., and the reaction mixture was diluted to twice its volume by gradual addition of a water solution containing a dispersant (1%) at 40° C. Purification was then effected by removing unreacted substances and sulfuric acid by means of dialysis in running water. A mixture was then formed of 3% of the finely-divided formalized polyvinyl alcohol of a degree of formalization of 50 mol percent thus obtained, sulfuric acid (10%) and  $\alpha$ -sodium sulfoacetaldehyde dimethylacetal (100 mol percent based on polyvinyl alcohol), and the mixture was stirred at 70° C. for 4 hours. Following purification by means of dialysis in running water, there was obtained a stable emulsion. The degree of sulfoacetalization of this emulsion was about 10 mol percent, and the particle diameter was about 1-5 $\mu$ . The emulsion was mixed with 10% of polyvinyl alcohol to produce a spinning solution having a total polymer concentration of 35%. Dry-spinning was effected in conventional manner by extruding the solution through a spinning nozzle of 0.3 mm. diameter into the air. The resultant fibers were stretched at 220° C. by 400%, and then relaxed at 225° C. by 15%. Upon benzalization by the procedure described in Example 2, fibers having a degree of benzalization of 24.5 mol percent were obtained. These fibers

40 (18.2 g.), polyvinyl alcohol (19.1 g.), ammonium per-sulfate (1.6 g.), sodium bisulfite (1 g.), and water (600 g.) at 60° C. After about 2 hours, the emulsion gradually coagulated, forming a precipitate. After further heating for 5 hours, the precipitate was dissolved in methanol, the solution poured into water, and the solids collected by evaporation. This process was repeated and there was recovered a copolymer containing allyl bromide (14.5 mol percent) in a yield of 56%. Twenty grams of this copolymer were heated with a 15% aqueous solution of sodium sulfite (180 g.) for 24 hours. Un-reacted substances were then removed by dialysis in running water, and the product was treated as described in Example 3 to produce a stable emulsion following purification dialysis. This emulsion was mixed with 15% of polyvinyl alcohol, and the spinning fluid thus produced were wet spun in conventional manner. The fibers were heat-treated and then formalized or benzalized as described in Example 2. All of the fibers thus obtained were found to have excellent dyeability.

#### Example 6

The procedure of Example 5 was repeated except that the allyl bromide copolymer was formalized in conventional manner prior to sulfonation by heating with the aqueous solution of sodium sulfite. A stable emulsion was obtained. This product was mixed with polyvinyl alcohol, and wet spun, and the fibers were heat-treated, and acetalized, as described in Example 5. Fibers exhibiting excellent dyeability with respect to various types of basic dyes were obtained.

#### Example 7

An aqueous solution containing polyvinyl alcohol (3%) sulfuric acid (15%) and a dispersant (2%) was stirred at 60° C., and benzaldehyde (50 mol percent based on polyvinyl alcohol) and o-sulfonylbenzaldehyde (20 mol percent based on polyvinyl alcohol) were gradually added. The product was purified by dialysis and there was ob-

5 6  
were dyed by means of Sevron Green B (4%) under the same conditions described in Example 2, whereby the fibers were dyed a bright, dark green color. The fibers showed an elasticity of 78% at an elongation of 3%, and had a feel which was very rich in elasticity.

#### Example 4

Substituting  $\alpha$ -carboxylacetaldehyde for  $\alpha$ -sodium sulfoacetaldehyde dimethylacetal, the procedure described in Example 3 was repeated and there was produced an emulsion of acetalized polyvinyl alcohol containing the carboxyl group. When this emulsion was mixed with polyvinyl alcohol, spun, heat-treated and benzalized as described in Example 3, fibers of high elastic were obtained which exhibited excellent dyeability with respect to various types of basic dyes. When the cross-section of the dyed fiber was examined microscopically, the presence of dyed fine particles was observed.

#### Example 5

20 Emulsion polymerization was effected by agitating a mixture composed of vinyl acetate (73 g.), allyl bromide

tained an emulsion of polyvinyl alcohol acetalized by benzaldehyde and o-sulfonylbenzaldehyde. This emulsion was mixed with 20% polyvinyl alcohol and the mixture was then spun and the fibers were treated in the manner described in Example 2. The fibers were found to have excellent dyeability.

*Example 8*

Using an emulsion of the copolymer of acrylonitrile containing sodium vinylsulfonate (15 mol percent), mixing with polyvinyl alcohol to form a spinning solution to form fibers, were effected in the manner described in Example 1. The fibers were then subjected to heat-treatment and formalization following the procedure of Example 1. Fibers having excellent dyeability with respect to basic dyes were obtained.

*Example 9*

A water solution containing chloroacetaldehyde (0.5%), formaldehyde (1%), polyvinyl alcohol (3%) and sulfuric acid (50%) was reacted and then diluted in the manner in Example 3. Acetalized polyvinyl alcohol containing halogen was thus obtained, in finely-divided form. This product was heated with a 10% aqueous solution of sodium sulfite to introduce the sulfo radical, and the reaction product was purified by dialysis. Following the procedure of Example 1, the product was mixed with polyvinyl alcohol, the mixture spun, and the fibers subjected to heat-treatment and formalization. There were obtained fibers exhibiting excellent dyeability for basic dyes.

The surface-active or dispersing agents or dispersants and protective colloids which are suitably employed are, in addition to those mentioned above, any of the many dispersing agents and protective colloids known to those skilled in the art of making emulsions or dispersions of polymers. In the foregoing examples, for instance, polyoxyethylenedodecyl ether is suitably used as the dispersant or surface-active agent.

It will be therefore be understood that, unless otherwise indicated, conventional operations and conventional apparatus are employed in carrying out the process of this invention including conventional mixing and emulsifying units. Similarly, conventional dyeing techniques and apparatus are suitably employed upon the fibers produced by the process of this invention. The conditions and the relative relationships set forth in the examples are those preferred in carrying out the process of the invention but it will be understood that other conditions and relationships may be used within the scope of the invention.

The spinning fluids produced in accordance with the present invention are particularly suitable for the spinning of fibers in accordance with known processes used in the spinning of polyvinyl alcohol and polyvinyl alcohol derivatives, particularly the so-called "wet-spinning" techniques as described, for example, in Cline et al. U.S. Patent 2,610,360 and Osugi et al. Patent No. 2,906,594. An especially preferred spinning technique is described in

copending application Serial No. 336,166 of Tomonari et al., filed February 10, 1953.

After formation of the fibers by wet spinning the filaments can, as mentioned, be further treated by stretching, heat treating, acetalization, and the like to produce fibers with desirable and outstanding properties. For such treatments known techniques such as described in said patents are suitably employed.

It will also be understood that various changes and modifications in addition to those indicated above may be made in the embodiments herein described without departing from the scope of the invention as defined in the appended claims. It is intended, therefore, that all matter contained in the foregoing description shall be interpreted as illustrative only and not as limitative of the invention.

I claim:

1. In the manufacture of polyvinyl alcohol fibers, the steps which comprise preparing an aqueous spinning fluid comprising a mixture of polyvinyl alcohol and a polymer containing a sulfonic acid group, said polymer being insoluble in said aqueous spinning fluid, dispersed in said aqueous polyvinyl alcohol spinning fluid in finely divided form and selected from the group consisting of homopolymers of an ethylenically-unsaturated monomer containing a sulfonic acid group, salts thereof, copolymers thereof with a second monomer selected from the group consisting of vinyl chloride, allyl chloride, vinylidene chloride, vinyl benzoate, allyl acetate, vinyl acetate, styrene, butadiene, divinylbenzene, methyl acrylate, methyl methacrylate, acrylonitrile, and methyl vinylketone, and polyvinyl alcohol acetalized by an aldehyde containing a sulfonic acid group, and spinning said fluid to form fibers therefrom.

2. The method as defined in claim 1 wherein the average quantity of said sulfonic acid group in said polymer is 1 to 70 mole percent and the average quantity of said polymer in said fluid is 0.1 to 10 mole percent based on the total polymer content of the fluid.

3. The method as defined in claim 1, wherein said ethylenically-unsaturated monomer containing a sulfonic acid group is a monomer selected from the group consisting of vinylsulfonic acid, allylsulfonic acid, and styrenesulfonic acid.

References Cited by the Examiner

UNITED STATES PATENTS

|           |        |              |         |
|-----------|--------|--------------|---------|
| 2,169,250 | 8/1939 | Izard et al. | 264—185 |
| 2,236,061 | 3/1941 | Izard et al. | 18—54   |
| 2,895,786 | 7/1959 | Shlack       | 18—54   |

OTHER REFERENCES

Hackh's Chemical Dictionary, 3rd ed., page 743  
(McGraw Hill Book Co., Inc.).

MURRAY TILLMAN, Primary Examiner.

D. ARNOLD, L. J. BERCOVITZ, Examiners.